

## UNITED STATES PATENT OFFICE

2,230,710

## PHOTOGRAPHIC PRINTING

Edith Weyde, Cologne-Niehl, Germany, assignor, by mesne assignments, to General Aniline & Film Corporation, New York, N. Y., a corporation of Delaware

No Drawing. Original application February 10, 1938, Serial No. 189,762, now Patent No. 2,205,756, dated June 25, 1940. Divided and this application December 16, 1938, Serial No. 246,067. In Germany February 15, 1937

8 Claims. (Cl. 95—88)

The present invention relates to an improvement in the production of photographic prints. This application is a division of my copending application Ser. No. 189,762 filed February 10, 1938, which matured into Patent No. 2,205,756, June 25, 1940.

Photographic papers have a tendency to adsorb and thus to retain sodium thiosulfate from the fixing baths and the soluble silver salts produced by the fixing operation. This phenomenon on the one hand affects the permanence of the photographic print since the retained salts gradually react with the silver image to form silver sulfide and the silver salts also gradually decompose into silver sulfide and thus impart a yellow tint to the paper; on the other hand the phenomenon leads to a more or less pronounced coloring of the whites in the toning of the print, particularly with a sulfide or a selenide, in consequence of the intensely colored silver salts which are formed.

The present invention is based on the observation that the barium sulfate used for whitening the paper is primarily responsible for the undesirable retention of the compounds or salts.

Precipitated barium sulfate has as is known the tendency to adsorb metallic salts (for instance  $BaCl_2$ ,  $MgCl_2$  or  $FeCl_3$ ) and other compounds particularly substances having a high molecular weight such as dextrin which itself has a strong adsorbing tendency (see, for instance, Marc, Zeitschrift für physikalische Chemie, 75, 710, 1911 and 81, 641, 1913). Moreover, it is known that the adsorbing a substance may be affected by adding a further component. The adsorbing Kongored by means of cellulose, for example, is intensely reduced by adding phosphate ions. It has also been proposed to remove mangano ions which are adsorbed by precipitated manganese dioxide with the aid of solutions of ferrous salts because manganese dioxide is capable of adsorbing ferro ions more intensely than mangano ions (Geloso, Ann. Chim. 6, 352, 1926).

It is one object of my invention to provide a process of removing sodium and silver thiosulfate being adsorbed by barium sulfate. Another object is the provision of a process of removing the thiosulfates by treating barium sulfate with substances having a strong tendency to become retained by adsorption.

Further objects will be apparent from the disclosure following hereinafter.

Particularly suitable for the purpose of the present invention are the salts of the rare earths.

It is noted that it is known that the hydroxides of the rare earths, the salt solutions of which as well known easily hydrolyze, are capable of adsorbing many substances.

It is immaterial at what stage in the manufacture and preparation of the paper these salts are allowed to act upon the barium sulfate. They may be added directly to the barium sulfate grounding or to the emulsion, from which they gradually migrate to the barium sulfate. The desired effect may also be obtained by using such salts in an intermediate bath following the development or as an addition to the fixing bath or even in a separate bath after fixing but before washing. The washing of the paper raw material which may contain the barium sulfate as filling agent may be improved by the substances so that it is advantageous to add them in the preparation of the paper. However, it is also practicable to soak the finished paper material with a solution of the substance.

It will be understood that in addition to the substances hereinbefore named there is a number of further substances which have the desired action. However, the use of these substances is in part restricted since it is necessary that there should be no coloration of the paper material or of the baytes and that the substance should not have an unfavorable effect on the photographic emulsion.

The following examples illustrate the invention:

(1) To 1 liter of a gelatin solution containing barium sulfate such as is used for coating the photographic paper, there are added 3 grams of lanthanum chloride.

(2) To a photographic emulsion there are added per liter 2 grams of cerous sulfate and the emulsion is applied to the paper in the usual manner.

(3) The photographic material is treated after development in a bath of the following composition:

|                     |       |      |
|---------------------|-------|------|
| Water               | cc    | 1000 |
| Glacial acetic acid | cc    | 10   |
| Thorium nitrate     | grams | 10   |

In this bath the photographic material remains for 1-10 minutes and is finally fixed.

I claim:

1. A photographic fixing material for photographic elements having a barite layer and a light-sensitive silver halide emulsion layer thereon, which comprises silver halide fixing agents and an amount of rare earth metal salt

sufficient to effectively suppress the absorptive capacity of the barite layer for thiosulfates.

- 5 2. In the process of producing photographic prints by exposing, developing, fixing with sodium thiosulfate and washing photographic paper having a barite layer and a light-sensitive silver halide emulsion layer thereon, the improvement which comprises immersing said photographic paper after the development thereof in a bath 10 containing an amount of a rare earth metal salt effective to suppress the adsorptive capacity of said barite layer for thiosulfates.
- 15 3. In the process of producing photographic prints by exposing, developing, fixing with sodium thiosulfate and washing photographic paper having a barite layer and a light-sensitive silver halide emulsion layer thereon, the improvement which comprises immersing said photographic paper after the development thereof in a fixing 20 bath containing an amount of a rare earth metal salt effective to suppress the adsorptive capacity of said barite layer for thiosulfates.
- 25 4. In the process of producing photographic prints by exposing, developing, fixing with sodium thiosulfate and washing photographic paper having a barite layer and a light-sensitive silver halide emulsion layer thereon, the improvement which comprises immersing said photographic paper after the development thereof in a bath 30 containing an amount of lanthanum

chloride effective to suppress the adsorptive capacity of said barite layer for thiosulfates.

- 5 5. In the process of producing photographic prints by exposing, developing, fixing with sodium thiosulfate and washing photographic paper 10 having a barite layer and a light-sensitive silver halide emulsion layer thereon, the improvement which comprises immersing said photographic paper after the development thereof in a bath containing an amount of thorium nitrate effective 15 to suppress the adsorptive capacity of said barite layer for thiosulfates.

- 15 6. In the process of producing photographic prints by exposing, developing, fixing with sodium thiosulfate and washing photographic paper 20 having a barite layer and a light-sensitive silver halide emulsion layer thereon, the improvement which comprises immersing said photographic paper after the development thereof in a bath containing an amount of cerous sulfate effective 25 to suppress the adsorptive capacity of said barite layer for thiosulfates.

- 25 7. A photographic stop bath comprising water, acetic acid and a water-soluble rare earth metal salt.

- 20 8. A photographic silver halide fixing bath comprising a thiosulfate and a rare earth metal salt.

EDITH WEYDE. 30